

[54] **METHOD FOR CHARGING PLASTIC POWDER ELECTROSTATICALLY BY FRICTION ONLY**

[76] Inventor: **Hans J. Schaad**, Erlenbachstrasse 37, 46 Dortmund-Schuren, Germany

[22] Filed: **Jan. 22, 1973**

[21] Appl. No.: **325,231**

[30] **Foreign Application Priority Data**

Jan. 25, 1972 Germany ..... 2203351

[52] **U.S. Cl.** ..... **427/25; 427/27; 239/15; 239/602; 239/DIG. 19; 317/3**

[51] **Int. Cl.<sup>2</sup>** ..... **B05B 5/02; B44D 1/094**

[58] **Field of Search** ..... 117/17; 317/3; 239/15, 239/602, DIG.19; 427/25, 27

[56] **References Cited**

UNITED STATES PATENTS

|           |         |           |       |
|-----------|---------|-----------|-------|
| 2,477,947 | 8/1949  | Yadoff    | 317/3 |
| 2,574,284 | 11/1951 | Prochazka | 317/3 |
| 2,590,534 | 3/1952  | Hampe     | 317/3 |
| 2,657,339 | 10/1953 | Hampe     | 317/3 |

|           |         |                  |          |
|-----------|---------|------------------|----------|
| 2,761,997 | 9/1956  | Forest et al.    | 117/17   |
| 3,339,841 | 9/1967  | Beach            | 239/15   |
| 3,434,859 | 3/1969  | Benjamin         | 117/17   |
| 3,507,686 | 4/1970  | Hagenbach        | 117/17.5 |
| 3,521,815 | 7/1970  | Szazs            | 239/15   |
| 3,533,835 | 10/1970 | Hagenbach et al. | 117/17.5 |
| 3,597,668 | 8/1971  | Yoshimine        | 317/3    |
| 3,630,442 | 12/1971 | Probst           | 239/15   |

*Primary Examiner*—Michael Sofocleous  
*Attorney, Agent, or Firm*—Fitch, Even, Tabin & Luedeka

[57] **ABSTRACT**

A method of coating particles with plastic material powder, such as epoxide resin powder without the use of an external electrical field comprises the steps of mixing the powder in a stream of pressurized air, accelerating the air and powder stream to supersonic velocity through a venturi device, electrostatically charging the plastic material powder by friction against a polytetrafluoro ethylene surface. The front portion of the nozzle discharging the material is grounded by a metallic sleeve.

**3 Claims, 3 Drawing Figures**



PATENTED SEP 2 1975

3,903,321

SHEET 1 OF 3



SHEET 2 OF 3



Fig. 2



## METHOD FOR CHARGING PLASTIC POWDER ELECTROSTATICALLY BY FRICTION ONLY

The present invention relates to a method of coating articles with plastic material powder, especially epoxide resin powder, in an electrostatic field, and an apparatus for carrying out such method.

It is well known to spray plastic material powder onto articles by means of accelerated air streams, whereby the particles of the plastic material powder are subjected to an electrostatic charge by an electrical field, so that they settle on the grounded or oppositely charged article because of the electrical attraction. Upon baking, the layer of plastic material powder provides a surface coating being superior to conventional lacquer coatings.

However, it is of disadvantage in the known powder coating methods and apparatuses that they require an electrostatic voltage source which, because of the high voltage used (between 30 and 150 kilovolts), necessitates expensive safety measures.

It is the object of the invention to provide a method and an apparatus for the powder coating of articles which do no longer show the abovementioned disadvantages and which, in particular, are more safe in operation, which render possible an ideal distribution of polarization and ionization which, otherwise, is disturbed by foreign charge, which are capable of operating without any additional voltage source for an electrostatic field, and wherein the apparatus is simple, easy and economical to manufacture and operate, and wherein it is possible to adjust the thickness of the coating by adjustment of the flow velocity or of the quantity of air, respectively.

According to the invention, this object is solved in that the plastic material powder is electrostatically charged by friction against polytetrafluoro ethylene (PTFE), and then sprayed onto the article to be coated.

Furthermore, the object according to the invention is solved in that the plastic material powder, after the self-charging by mutual friction between the plastic material particles and/or with the nozzle walls, is further passed through highly insulating materials only which, preferably, have a very high resistivity of about from  $10^{16}$  to  $10^{20}$  ohms per centimeter.

In a manner being particularly surprising to the expert, it has shown that the good coating according to the invention can be obtained not only by using polytetrafluoro ethylene, but that, further, polytrifluoro monochloroethylene and other fluoro compounds and solid, highly insulating materials, such as amber, mica and quartz glass, may be employed.

Prior condition for the usability is, on the one hand, a high insulating effect which substantially exceeds the insulating effect of e.g. standard glass and the like, and, on the other hand, a surface consistency which safely prevents the plastic material powder from adhering thereto. Additionally, the material must be chemically inert towards the plastic material powder, too.

In the following, an exemplary embodiment of the invention is explained in greater detail by referred to the accompanying three drawings.

FIG. 1 schematically shows in sectional view an apparatus for discharging electrostatically charged plastic material powder, whereby the powder reservoir is attached directly to the jet pipe.

FIG. 2a pistol for the powder coating of articles according to FIG. 1 and

FIG. 3a pistol according to FIG. 2 but without having the powder supply attached to the pistol.

The powder spraying apparatus according to the invention comprises primarily a jet pipe 1 and a mixing section 2 positioned upstream thereof, both components being formed of polytetrafluoro ethylene. The jet pipe 1 per se may consist of a nozzle portion 1c having a subsequent expansion portion 1b which is followed by the actual spray pipe 1a. The spray pipe 1a may merge with a diffusor 7 wherein the velocity of the outflowing powder/air mixture is lowered, and includes a perforated plate 6 which is likewise formed of polytetrafluoro ethylene and which provides a uniform flow distribution.

15 The powder enters the mixing portion 2 which preferably is a cylindrical chamber, via a passage 8. The passage 8 may be either directly surrounded by a powder reservoir 9, (FIG. 2), or the powder may be fed thereto over a certain distance (FIG. 3).

20 The rear wall of the mixing or distributor section 2 includes an opening into which a nozzle housing 4 opens. The nozzle housing which likewise consists of polytetrafluoro ethylene, has a nozzle needle passing coaxially therethrough, whereby the quantity of the entering air may be controlled by the position of this needle. Of course, it is also possible to introduce the air via the nozzle housing 4, whereby the quantity of air may be adjusted at some distance, e.g. in the pressurized air feed conduit. In such case, the nozzle needle may be omitted.

25 The apparatus according to the invention may be formed either as a hand spray gun by being provided with a handle 11 or it may be positioned with some distance from the powder reservoir either stationarily or so as to be movable (FIG. 3).

30 It is important for the generation of a very high electrostatic field of e.g. up to 200 kilovolts that the whole quantity of powder within the accelerated air flow may contact the polytetrafluoro ethylene only, so that, on the one hand, there are produced ionized and polarized powder particles, and, on the other hand, the resulting charges are not dissipated afterwards.

35 In a manner being surprising to the expert, the self-charging of the powder particles renders possible both a polarization and an ionization of the powder particles in ideal combination, so that, when selecting high flow velocities, high thicknesses of the coating in comparison with conventional coating methods may be obtained.

40 By adjustment of the flow velocity, the deposition of the powder particles may be controlled, so that smaller layer thicknesses may be adjusted, too.

45 By forming the nozzle with a minimum cross-sectional area and a subsequent expansion zone within the extension of a continuous curvature, it is possible to produce supersonic flow velocities.

50 Surprisingly, the use of polytetrafluoro ethylene in combination with the flow velocity does not only result in that a voltage source becomes superfluous, but also, as mentioned above, in that a superior coating is obtained.

55 The charging and, thus, the coating depend on the temperature and on the humidity of the pressurized air. Therefore, it is advisable to provide for a pre-drying of the air when operating at high humidity. However, it has been found that an adequate coating by means of

the method according to the invention can be obtained even at very high humidities (of above 90%).

Epoxide resin is particularly useful for the processing in accordance with the present method. It has been found, however, that polyester, polyamide and other plastic material powders can be processed with good results, too, by using the method according to the invention.

Surprisingly, the electrostatic properties of polytetrafluoro ethylene are superior to any other plastic materials. Enclosed is a Table showing the surprising effect obtained in the processing of various types of plastic materials when using jet pipes and mixing chambers made of polytetrafluoro ethylene. Evidently, a coating can still be obtained when using polyethylene; however, the use of polytetrafluoro ethylene results in a improved effect which is absolutely unexpected by the expert and which, in view of the previous knowledge about the effect of plastic parts in powder spray guns, could not be foreseen, which fact is also demonstrated by the submitted compilation.

In order to obtain the effect according to the invention, it is essential that all portions of the mixed flow of driving air and powder are in contact with polytetrafluoro ethylene surfaces only, and that a sufficiently high flow velocity within the jet pipe is produced by using driving air of high pressure.

Apparently, sonic flow velocity and supersonic flow velocity may be adjusted with the apparatus according to the invention formed in the manner of a Laval nozzle, already by using driving air having a pressure of more than 2 atmospheres.

Advantageously, at least the front portion of the jet pipe 1 is surrounded by a grounded metallic sleeve 3 in order to prevent annoyance of the operators by spark generation on the surface of the jet pipe. Furthermore, this metallic sleeve 3 provides a certain improvement of the effect according to the invention.

If spreading device 12 is mounted within the nozzle 14 of jet pipe 1 e.g. by means of ribs 13, this spreading device as well as the ribs and the nozzle 14 should consist of polytetrafluoro ethylene. According to FIGS. 2 and 3 jet tube 1 may be covered by an outer protective sleeve 15 made of PVC or the like. According to FIGS. 2 and 3 switch 16 within the handle ii via a cable 17 by means not shown controls supply of pressurized air flowing to the pistol through flexible tube 19 and via removable nozzle 18, being screwed into the pistol

housing. In case of the pistol according to FIG. 3, where coating powder is supplied via tube 8, the control of the powder supply is effected by switch 16 as well.

Referring now to the following table, a number of experiments were performed with apparatus constructed in accordance with the drawings using several different materials or a combination of materials for the Venturi nozzle 1c. Also, several types of powder including epoxide powders were used with the apparatus of the various materials in attempting to determine the best combination of materials and powders for use with the illustrated apparatus. It was discovered that the use of polytetrafluoro ethylene, particularly when using epoxide powders produced the best results. The coating formation on the article sprayed was also analyzed.

More specifically, an electrostatic measuring instrument was used to measure the charge of the powder particles in micron amperes. When teflon is used for the apparatus, the average charge was at least one micron amp and for the epoxide powders, the charge was even 1.5 to 2.5 micron amps as shown in the Table.

Referring more particularly to the Table, it will be seen that first Column is labeled "Teflon" has a first subcolumn with numerals showing the micron amperes ( $\mu$ A) measured by the electrostatic measuring instrument for the various powders. Thus, the first five epoxide powders measured at least one micron amp charge. In contrast thereto, when using such materials as PVC or polycarbonate or polypropylene for the Venturi tube the average charge of the powder was less than 1 and in many cases zero.

The coating formations were also analyzed and rated during these experiments. A very good coating formation is indicated in the Table by a numeral 1 in the second sub-column under the letter S which refers to coating formation. Thus, the first five epoxide powders had a very good coating formation only when Teflon was used for the Venturi nozzle. Several other powders had a good coating formation as indicated by the numeral 2 when using Teflon. In contrast, the PVC, polycarbonate and polypropylene coatings generally were labeled 3's, 4's, and 5's, with 3 being only "usable", 4 being "not usable" and 5 indicating "no adhesion" at all. Thus, it is readily apparent that surprising and superior results were obtained by using Teflon and epoxide powders as set forth in the first upper left hand portion of the Table.

TABLE

| TYPE OF POWDER        | Coating Formation (S) |                         | Current ( $\mu$ A) and Coating formation (S) with Venturi nozzles made of various materials and with the use of different powders |                |                        |                         |                           |                           |                          |                           |     |   |   |   |
|-----------------------|-----------------------|-------------------------|-----------------------------------------------------------------------------------------------------------------------------------|----------------|------------------------|-------------------------|---------------------------|---------------------------|--------------------------|---------------------------|-----|---|---|---|
|                       | Teflon<br>$\mu$ A     | Glass-Teflon<br>$\mu$ A | Graphite-Teflon<br>$\mu$ A                                                                                                        | PVC<br>$\mu$ A | Hard Rubber<br>$\mu$ A | Polyethylene<br>$\mu$ A | Poly-carbonate<br>$\mu$ A | Poly-propylene<br>$\mu$ A | Poly-urethane<br>$\mu$ A | Aluminum Metal<br>$\mu$ A |     |   |   |   |
|                       | S                     | S                       | S                                                                                                                                 | S              | S                      | S                       | S                         | S                         | S                        | S                         | S   | S | S | S |
| Epoxide Standard      | +1.5                  | 1                       | +1                                                                                                                                | 1              | +0.5                   | 2                       | +                         | 4                         | +                        | 3                         | 0.5 | 2 | 0 | 4 |
| Epoxide Graphite      | +2                    | 1                       | +1.5                                                                                                                              | 2              | 0                      | 3                       | 0                         | 4                         | 0                        | 3                         | 0   | 3 | 0 | 3 |
| Epoxide Black         | +1                    | 1                       | +1                                                                                                                                | 2              | +1                     | 2                       | 0                         | 4                         | 0                        | 3                         | 0   | 4 | 0 | 5 |
| Epoxide Metal         | +1                    | 1                       | +1                                                                                                                                | 2              | +0.5                   | 3                       | 0                         | 3                         | 0                        | 4                         | 0.5 | 2 | 0 | 5 |
| Epoxide White         | +2.5                  | 1                       | +0.5                                                                                                                              | 2              | +1.5                   | 1                       | +0.5                      | 2                         | +0.5                     | 2                         | +1  | 1 | 0 | 3 |
| Polyester Thermoplast | +0.5                  | 4                       | +1.5                                                                                                                              | 2              | +1.5                   | 2                       | 0                         | 5                         | 0                        | 5                         | 0   | 0 | 5 | 0 |

TABLE -Continued

## Coating Formation (S)

1 = very good  
2 = good  
3 = still usable  
4 = not more usable  
5 = no adhesion

Current ( $\mu$ A) and Coating formation (S)  
with Venturi nozzles made of various  
materials and with the use of different  
powders

| TYPE OF<br>POWDER     | Teflon  |   | Glass-<br>Teflon |   | Graph-<br>ite-<br>Teflon |     | PVC     |       | Hard<br>Rubber |   | Poly-<br>ethylene |   | Poly-<br>carbonate |   | Poly-<br>propylene |   | Poly-<br>ure-<br>thane |   | Alu-<br>minum<br>Metal |   |
|-----------------------|---------|---|------------------|---|--------------------------|-----|---------|-------|----------------|---|-------------------|---|--------------------|---|--------------------|---|------------------------|---|------------------------|---|
|                       | $\mu$ A | S | $\mu$ A          | S | $\mu$ A                  | S   | $\mu$ A | S     | $\mu$ A        | S | $\mu$ A           | S | $\mu$ A            | S | $\mu$ A            | S | $\mu$ A                | S | $\mu$ A                | S |
| Polyester,<br>curable | 0       | 5 | 0                | 5 | -1.5                     | 2   | -       | 5     | -              | 5 | 0                 | 5 | -                  | 5 | -                  | 5 | -                      | 5 | 0                      | 5 |
| Polyester             | 0       | 3 | 0                | 4 | 0                        | 470 | 3       | +0.53 | 0              | 4 | 0                 | 3 | 0                  | 4 | +0.52              | 0 | 5                      | 0 | 5                      |   |
| Polyester             | +5      | 2 | +4               | 2 | +0.5                     | 3   | 0       | 5     | 0              | 5 | 0                 | 4 | 0                  | 5 | 0                  | 5 | 0                      | 5 | 0                      | 5 |
| Polyamide             | +1      | 2 | +0.5             | 2 | +0.5                     | 3   | +1      | 2     | +0.5           | 2 | +1                | 2 | +1                 | 2 | +1                 | 2 | 2                      | 2 | 0                      | 5 |
| PVC                   | +0.5    | 3 | +0.5             | 4 | +0.5                     | 4   | 0       | 5     | 0              | 5 | -0.5              | 2 | 0                  | 5 | 0                  | 5 | 0                      | 5 | 0                      | 5 |
| Polyurethane          | +0.5    | 3 | +0.5             | 3 | +1                       | 2   | 0       | 5     | 0              | 5 | 0                 | 5 | 0                  | 5 | 0                  | 5 | 0                      | 5 | 0                      | 5 |

+ = positive;

- = negative;

0 = no indication

I claim:

1. A method of coating articles with an epoxide powder within an electrostatic field without applying an external charge to the article comprising the steps of: mixing the epoxide powder in a stream of pressurized air within a mixing section of polytetrafluoro ethylene, accelerating the air and powder stream to supersonic velocity through a venturi device of polytetrafluoro ethylene, electrostatically charging the material powder solely by friction of the material flowing against the polytetrafluoro ethylene in said venturi device, passing the charged powder through a spray device having a surface of polytetrafluoro ethylene to prevent dissip-

ation of the charges on said particles, and discharging and spraying the electrostatically charged epoxide powder from the spray device onto the article to be coated.

2. A method in accordance with claim 1 including the step of: grounding a nozzle from which the spray is discharged.

3. A method in accordance with claim 1 including the step of providing the epoxide powder in a powder reservoir and feeding the epoxide powder for mixing in the stream of pressurized air within the mixing section.

\* \* \* \* \*

35

40

45

50

55

60

65